

## UNITED STATES PATENT OFFICE

2,338,917

## PROCESS FOR MANUFACTURING ARTIFICIAL TEXTILE FIBERS FROM CASEIN

Antonio Ferretti, Milan, Italy; vested in the  
Allen Property CustodianNo Drawing. Original application February 17,  
1938, Serial No. 191,000. Divided and this application April 20, 1940, Serial No. 330,727. In Italy March 2, 1937

8 Claims. (CL 18—54)

The present invention has for its object an embodiment in the process for manufacturing artificial textile fibers from animal casein.

The process according to the invention includes (1) spinning filaments from an alkaline solution of animal casein and coagulating the same in acid baths and (2) rendering the filaments insoluble at a temperature above 25° C. (twenty-five) and about 70° C. (seventy) in bath of formaldehyde to which soluble salts have been added, to render the filaments boilingproof.

The invention includes also (1) spinning filaments from a solution of animal casein and coagulating the same in acid baths (2) hardening the coagulated filaments by passing them through baths containing soluble salts at a temperature above 25° C. (twenty-five) and about 40° C. and (3) cutting the hardened filaments to the desired length and then insolubilising the fibers at a temperature above 25° C. and about 70° C. in baths of formaldehyde to which soluble salts have been added.

Specifically, the invention includes (1) spinning filaments from a solution of animal casein and coagulating the same in acid baths (2) hardening the filaments by passing the same firstly through a bath of sodium chloride at a temperature above 25° C. and about 40° C. and then through a bath containing aluminium salts and sodium chloride at a temperature above 25° C. and about 55° C. and (3) cutting the hardened filaments to the desired length and insolubilising the fibers at a temperature above 25° C. and about 70° C. in baths of formaldehyde to which soluble salts have been added.

Furthermore the invention includes (1) spinning filaments from a solution of casein, coagulating the same, in acid baths, insolubilising the same at low temperatures and (2) treating the filaments insolubilised at low temperatures with solutions of formaldehyde at a temperature above 25° C. and about 70° C. to render the same boiling-proof.

This application is a division of copending previously filed parent application Serial No. 191,000, filed February 17, 1938; said parent application, and therefore the present application, being based upon the earlier filing of corresponding application in Italy on March 2, 1937, which Italian application has subsequently resulted in Italian Patent No. 367,405, granted January 24, 1939.

The invention will be now explained with reference to the example of carrying out into practice.

In the manufacture of fibers of casein in which an initial immersing bath for the filaments is provided, said immersion bath for the filaments being composed of sodium chloride or other salts and a preparatory bath for rendering the fibers insoluble or a complete bath for rendering the fiber insoluble it is of great importance that the bath's temperature be not below 25° C. The temperature must be preferably between 35° C. and 40° C. for the first bath of sodium chloride or other salts and between 50° C. and 65° C. for the preparatory bath for rendering the fibers insoluble, of aluminium salts, sodium chloride or for the complete bath for rendering the fibers insoluble of formaldehyde, aluminium salts and sodium chloride or other salts.

It is also important that the temperature in the bath, in which the fibers as soon as cut are introduced be not below 25° C., it being preferable to employ a temperature between the range 35° C. to 40° C.

The treatment for rendering the casein fibers insoluble extends over a very long period, even several days, when carried out in a bath at ambient temperature, which is usually less than 25° C., nevertheless the fibers offer little resistance to boiling extending over a long period. On the contrary, it is found that when the temperature of the baths for rendering the fibers insoluble is raised for example to between 60° C. and 70° C., perfect insolubility is obtained in less than nine hours, and the fiber which has been treated at that temperature completely resists boiling which may extend over many hours. Before proceeding to this strong treatment it is preferable to pass the fibers for some hours into the collecting bath of the cut fibers at a temperature of between 35° C. and 40° C.

Complete resistance to the extensive boiling could also be obtained, when the casein fibers which have been rendered insoluble at a temperature which is lower than that indicated, for instance at 25° C. to 50° C., are treated, preferably after being washed and dried, with an aqueous solution of formaldehyde at a temperature of about 60° C. to 70° C. for several hours, for example, five hours. In this case, the addition of the aluminium salts, of sodium chloride or of other soluble alkaline metal salts or earthy alkalies, to the formaldehyde solution, is unnecessary.

This treatment could be effected with the dried casein fibers at any desired time, that is to say, even after a period of many months or years from the manufacturing date of the fiber has elapsed.

Above all, it is of great importance that the

treatment for rendering the fibers insoluble should be effected at temperatures which are not below 25° C., and that, when a temperature above 25° C., is applied, the relative operation should take place in an autoclave (digester) which should preferably be rotary, so as to maintain the fibers in motion while at the same time, the bath for rendering the fibers insoluble is made to circulate in the interior of the autoclave.

The further particulars of the manufacturing process for the textile fibers of casein may be modified in various ways without departing from the spirit of the invention.

The invention can also be applied to the manufacture of mixed fibers of casein and cellulose.

Of course the invention also covers the textile fibers of casein obtained by the indicated process.

Having now particularly described and ascertained the nature of my said invention and in what manner the same is to be performed I declare that what I claim is:

1. In a process for the manufacture of artificial textile fibers from casein and following the stage of spinning a multiplicity of filaments from an alkaline solution of the casein and coagulating them in an acid coagulating bath; the steps of aftertreating the delicate coagulated filaments comprising initially hardening them in an aqueous bath containing at least one soluble aluminum salt, and then subjecting the hardened filaments to the insolubilizing action of an aqueous formaldehyde bath maintained at a temperature between about 25° and 70° C., thereby to render the resulting casein fibers proof against impairment under boiling temperature.

2. The process as in claim 1 and wherein the initial hardening bath contains also sodium chloride and is maintained at a temperature between about 35° and 40° C.

3. The process as in claim 1 and wherein following the initial hardening bath the filaments are treated in a second aluminum salt hardening bath, containing sodium chloride, and maintained at a temperature between about 50° and 65° C.

4. In a process for the manufacture of artifi-

cial textile fibers from casein and following the stage of spinning a multiplicity of filaments from an alkaline solution of the casein and coagulating them in an acid coagulating bath; the steps of aftertreating the delicate coagulated filaments comprising hardening them in an aqueous bath containing at least one soluble aluminum salt, and then insolubilizing them in an aqueous formaldehyde bath maintained at a temperature between about 60° and 70° C.

5. A process as in claim 4 and wherein the insolubilizing bath contains both a soluble aluminum hardening salt and sodium chloride.

6. In a process for the manufacture of artificial textile fibers from casein and following the stage of spinning a multiplicity of filaments from an alkaline solution of the casein and coagulating them in an acid coagulating bath; the steps of aftertreating the delicate coagulated filaments comprising initially hardening them in an aqueous bath containing at least one soluble aluminum salt and maintained at a temperature of above 25° C., and then subjecting the hardened filaments to the insolubilizing action of a preliminary aqueous formaldehyde bath maintained at a temperature between about 35° and 40° C., and thereafter to a final insolubilizing bath of formaldehyde maintained at a temperature of about 60° to 70° C., thereby to render the resulting casein fibers proof against impairment under boiling temperature.

7. The process as in claim 6 and wherein after the hardening bath the filaments are cut to length before treatment in the preliminary insolubilizing bath.

8. In a process for manufacturing artificial textile fibers from an alkaline solution of casein the step, following spinning and acid coagulation of the casein filaments, and preceding insolubilizing the filaments by formaldehyde, of treating the freshly coagulated filaments in at least one aqueous bath at a temperature of about 40° C. in which bath at least one salt has been dissolved taken from the group consisting of water-soluble salts of alkaline metals and of alkaline earth metals.

ANTONIO FERRETTI.